

A. L. CLAPP,  
TRANSFER SHEET AND METHOD OF FORMING SAME,  
APPLICATION FILED JULY 16, 1914.

1,280,399.

Patented Oct. 1, 1918.

Fig. 1.



Fig. 2.



Fig. 3.



Fig. 4.



Witnesses:

James R. Hodder  
R. G. Hensley

Inventor:

Albert L. Clapp,  
by Geo. S. Maxwell, Attorney.

# UNITED STATES PATENT OFFICE.

ALBERT L. CLAPP, OF BRAINTREE, MASSACHUSETTS.

## TRANSFER-SHEET AND METHOD OF FORMING SAME.

1,280,399.

Specification of Letters Patent.

Patented Oct. 1, 1913.

Application filed July 16, 1914. Serial No. 551,349.

*To all whom it may concern:*

Be it known that I, ALBERT L. CLAPP, a citizen of the United States, and resident of Braintree, county of Norfolk, State of Massachusetts, have invented an Improvement in Transfer-Sheets and Methods of Forming Same, of which the following description, in connection with the accompanying drawings, is a specification, like letters 10 on the drawings representing like parts.

My present invention is an improved means of transferring or embossing and stenciling in gold, silver, bronze, colors, black or white, whereby the name, design, or 15 the like may be stamped in the desired color directly on an article. My invention is especially valuable for use in embossing or stenciling firm names, trademarks, and the like on leather, shoes, books, or on cloth, canvas, 20 silk, or satin materials, such as the linings of clothing, gloves, hats, etc. My invention, broadly considered, comprises a thin paper strip, adapted to receive and carry the gold, silver or color which it is desired to emboss 25 on letters or design or any work, which strip will enable the letters or design to be stamped directly on the article by the application of a suitably heated die. Heretofore it has been necessary in embossing or 30 stenciling, to specially treat the surface of the work to which letters or a design were to be applied, such treating consisting in applying sizing or the like, then the gold leaf, chalked paper, or similar metal leaf was 35 laid on the work, and by means of a die stamped and countersunk therein. By means of my present invention I provide a prepared embossing strip, containing any desired color chemically compounded so as 40 to adhere directly on to the work without special sizing or the like, and which color also will leave the paper strip carrying it freely, clearly and cleanly, substantially all such color being transferred from the carrying 45 strip directly on to the work. Furthermore by the present invention, I am enabled to utilize waterproof colors, which thereby secure permanency to the embossed design, and by provision of means for the colors 50 to leave the carrying strip clearly, a brilliancy in the embossed work is insured.

A further important feature of my present invention is that a paper strip or carrier for the colors is so prepared as to be flexible and 55 may therefore be rolled on spindles, folded if desired, and of course may be handled

without danger of the colors carried by such strip being damaged or coming off of the strip. To this end I chemically compound the colors so as to leave the paper strip on 60 which they are spread only under the influence of heat and pressure, such heat and pressure being applied to the reverse side of the paper strip by means of a suitable die, which die carries the design, letters, or 65 70 like, intended to be embossed on the work.

The advantages incident to my invention of a strip carrying chemically prepared and inherently adhesive colors for embossing 70 purposes, will be readily appreciated when it is realized that heretofore it has been customary to use chalk colors on paper sheets, which sheets had to be kept flat, wherein the colors easily rubbed off in han- 75 dling, were difficult to transport or keep, and which also required special treating, sizing, or the like, of the work before the colors could be applied thereto. A similar objection in the prior use of gold leaf, silver 80 leaf, or other metal leaf, was present, since such sheets are easily spoiled by folding, or even falling to the floor, must be most carefully handled and can only be packed flat for keeping or shipping and also require 85 separate sheets of tissue or the like covering each leaf. My chemically prepared compound, on the contrary, is flexible, may be folded, and is not damaged by falling on the floor or handling, and is adhesive to the 90 work without coating either the work or the color to be applied with sizing, glue, or the like.

The first step for preparing the paper strip or carrier is to prepare one surface 95 with any suitable filler or coating, such as dextrin, to prevent the color compound from permeating the paper strip applied to that side, and furthermore to insure that the color compound will all leave the paper 100 strip in a clear, clean, sharp manner when the heated die is applied thereto. The color compound is then spread upon the side of the paper sheet or strip so prepared in a heavy or light coat, as best suited for the 105 particular work in hand, and as soon as the strip is dry it is ready for use. In use, the colored strip is applied with the colored side downwardly upon the work to be stenciled, embossed, or stamped, and a sufficiently 110 heated die is applied to the reverse side of the paper strip. The heat and pressure

transfers the chemically prepared color compound on the lower side of the strip directly to the work. I so prepare the color compound that it will adhere to the paper strip, excepting only when subjected to heat and pressure on the reverse side, and when so subjected it will at once become plastic, sticky, or the like, and adhere directly to the work adjacent thereto or on which the strip 5 may rest.

It will be readily appreciated that I may chemically prepare a color compound in a variety of ways and of a great variety of proportions, the important feature of my 10 invention being that the color,—gold, silver, red, blue, bronze, black or white, may be compounded either from dye or pigments, together with such ingredients as will render the compound adhesive under the application of heat and pressure, and readily 15 transferable from a thin paper strip to the work, and to permanently adhere to said work so transferred. I have successfully transferred various colors to leather, to fabric, 20 canvas, satin, silk, and the like, as well as to wood pulp, glass, and many other articles. Even greasy or oily leather and glazed leather, which have heretofore been very difficult to emboss by any means, may be 25 readily stamped and will permanently hold letters, designs, or the like embossed with my compound as above explained.

Referring to the drawings, illustrating my colored strip and the manner of embossing 30 therefrom,

Figure 1 is a fragmentary view of the embossing strip, showing the same after two impressions have been taken therefrom, as well as a portion of the unused strip;

Fig. 2 is a view in cross section, considerably enlarged, to show that the coloring compound may be carried clear to the edge of the strip;

Fig. 3 is a plan view of trademark lettering stamped from my strip; and

Fig. 4 is a view of the lettering shown in Fig. 1 and stamped therefrom on a book cover.

The paper strip 1 is coated with my 50 chemically prepared compound 2 as will be explained, this compound being of any desired color, as well as gold, silver, bronze, or the like. In using the same, the prepared side 2 is laid face downward upon the work, as, for example, the heel pad 3, or the book cover 4, and a heated die is then brought 55 into contact on the uppermost surface of the paper 1, the heat and pressure at once transferring the colored coating 2 on to the work 60 wherever the die is applied. The coating, being inherently composed of sufficient adhesive, adheres to the work, transferring all the coloring compound from the particular portion under the die being used. The 65 trademark 5 illustrated in Fig. 4 and

stamped from the embossing sheet shown in Fig. 2, leaving the corresponding blanks, as indicated at 6 in said sheet, may thus be readily transferred. After this trademark has been stamped, a different design, such 70 as the trademark 7 shown in Fig. 3, may be stamped, or any other desired lettering, mark, stenciling, or design, and in such colors as is desired.

In preparing the compound, I find that a 75 considerable leeway is feasible in the formula used, and for the particular work desired, but in color work, for example, I find that the following formula gives very satisfactory results, *i. e.*, 6 cc. amylacetate, 2 gr. 80 rosin, 1 cc. linseed oil,  $\frac{1}{2}$  gr. nitro-cellulose, 4 gr. bronze powder, all thoroughly mixed together, and then applied to the sheet of paper in an even coating by brush, or flowing it on to the paper. One of the important features of the rosin is to make the compound leave the paper cleanly and fully, and also lowering the melting point of the entire coloring compound, softening it sufficiently so that it will fuse under light heat 85 and pressure and be transferred to the work. Instead of 4 gr. bronze powder, I can use the foregoing formula by substituting 6 gr. coloring pigment with good success. In making a red compound, for example, I may use 40 cc. of carbon tetrachlorid, 7 gr. rosin dissolved therein, 2 gr. ceres red, and add a slight amount of adhesive, thoroughly mix the compound and apply the same to the paper and it will be readily transferred under heat and pressure as 90 above explained. In preparing a blue coloring compound, for example, I employ 40 cc. alcohol, 7 gr. rosin, 4 gr. ceres blue, 2 gr. dry shellac, and a small amount of adhesive, such as 1 gr. nitro-cellulose, and mix thoroughly together and apply to the paper strip. In preparing my embossing strip for use on oily leather or glazed leather, it may 95 be desirable to also mix in a small amount of dry dextrin, the amount varying with the work in hand.

The foregoing formulæ will be sufficient to treat 20 yards of 1 inch wide embossing strip for ordinary work, and, of course, it 100 will be understood that any dyes or pigments to secure different colors may be employed, or a combination of a dye and pigment may be utilized. The important feature of the invention, broadly considered, is to provide 105 an embossing strip coated with a chemically prepared compound, having sufficient adhesive to enable the same to be transferred directly to the work, without specially preparing the work, and to be so transferred 110 under heat and pressure. It will also be understood that, in employing dyes where a solvent is employed to aid in thinning the compound for treating or coating the strip, the solvent will then evaporate and leave the 115 120 125 130

residue free thereof, and I wish to claim this feature of the invention. In employing a pigment, however, it will doubtless be advisable to use some liquid thinning medium which will not necessarily dissolve the pigment, but merely hold it in suspension to facilitate the coating operation, and such thinning medium will then evaporate after a proper period of time. I wish, therefore, 10 to cover broadly my invention, either when the solution or thinning medium has evaporated, or before it has evaporated, as in either instance the strip may be used.

Having described my invention, what I 15 claim as new and desire to secure by Letters Patent is:

1. An article of manufacture comprising a paper backing, and a coating of chemically prepared color compound including amyl- 20 acetate, rosin, linseed oil, nitro-cellulose,

and colored powder mixed together and applied to one side of the backing, whereby a design may be transferred from said backing by the application to the uncoated side of a heated die.

25

2. An article of manufacture, comprising a paper strip, and a coating on one side of said strip of a chemically prepared solution, comprising 6 cc. amylacetate, 2 gr. rosin, 1 cc. linseed oil, one-half gr. nitro-cellulose, 30 and 4 gr. colored powder, mixed together and applied to said strip.

In testimony whereof, I have signed my name to this specification, in the presence of two subscribing witnesses.

ALBERT L. CLAPP.

Witnesses:

JAMES R. HODDER,  
R. G. HERSEY.